

## UNITED STATES PATENT OFFICE

RAINALD BRIGHTMAN, OF BLACKLEY, MANCHESTER, ENGLAND, ASSIGNOR TO IMPERIAL CHEMICAL INDUSTRIES LIMITED, OF LONDON, ENGLAND

## DYEING OF REGENERATED CELLULOSE MATERIALS

No Drawing. Application filed April 17, 1930, Serial No. 445,227, and in Great Britain April 19, 1929.

According to this invention the secondary disazo dyestuffs obtained by coupling a diazotized amine of the benzene series with an amino-naphtholsulphonic acid in alkaline solution, diazotizing the aminoazo dyestuff obtained and coupling with a suitable coupling component, are used for the production of even dyeings on regenerated cellulose rayon. The dyestuffs so obtained give shades varying from orange and red to bluish violet or blue and are characterized by the valuable property of dyeing viscose rayon in even shades. Certain dyestuffs of the aforesaid type are already known but they have not been described for the dyeing of viscose rayon and in particular it was not foreseen that they would have the valuable property of dyeing viscose rayon in even shades.

I have found that regenerated cellulose materials may be dyed in even level shades by means of secondary disazo dyestuffs which may be represented by the following generic formula:



wherein  $\text{R}_1$  represents a coupled residue of a diazotized amine of the class consisting of chlor-aniline, amino-benzoic acid and anisidine,  $\text{R}_2$  represents a naphthalene residue and  $\text{R}_3$  represents a coupled residue of an azo dye coupling component of the class consisting of beta-naphthol, nitro-m-phenylene diamine, salicylic acid and amino-naphthol sulphonic acids and  $x$  is 1 or 2. Within this generic class of dyes there are several subgeneric classes which are especially advantageous for dyeing regenerated cellulose materials in even level shades. The following structural formulae indicate certain of these subgeneric classes which are typical. 40 In the following formulæ  $\text{R}_1$ ,  $\text{R}_2$ ,  $\text{R}_3$  and  $x$  have the same significance as above.

50





12 by diazotizing 1 mol. of p-chloroaniline, coupling in alkaline solution with 1 mol. of 2-amino-8-naphthol-6-sulphonic acid, diazotizing the resultant aminoazo dyestuff and coupling in alkaline solution with 1 mol. of 2-amino-8-naphthol-6-sulphonic acid. 100 parts of the regenerated viscose rayon are entered into the bath warm and the bath is then raised nearly to the boil and the dyeing carried on for about  $\frac{3}{4}$  hour. The fabric is then removed, rinsed and dried. Alternatively, the rayon may be entered into the bath nearly at the boil and allowed to cool gradually during the dyeing. Moreover, there may be also used in the dyebath, other salts or dyeing assistants, as borax. The rayon is dyed a violet brown shade. 70  
 13 75

the subgeneric classes given generic classes which may be by the following structural formulae following generic formulæ, X hydrogen or a sulphonic group, is chlorine, an alkoxy or a car- and the other symbols have the

The invention is further illustrated by the examples in the following table: 80

85

| Component | Middle component (alkaline coupling)                                                                                                                                                                                                                                                                         | End component (all couplings with amino-naphthol sulphonic acid are in alkaline solution)                                                                                                                                                                                                                       | Shade on viscose rayon                                                                                                                  |
|-----------|--------------------------------------------------------------------------------------------------------------------------------------------------------------------------------------------------------------------------------------------------------------------------------------------------------------|-----------------------------------------------------------------------------------------------------------------------------------------------------------------------------------------------------------------------------------------------------------------------------------------------------------------|-----------------------------------------------------------------------------------------------------------------------------------------|
| 12        | 2-amino-5-naphthol-7-sulphonic acid<br>Do.<br>2-amino-8-naphthol-6-sulphonic acid<br>Do.<br>Do.<br>1-amino-5-naphthol-7-sulphonic acid<br>2-amino-5-naphthol-7-sulphonic acid<br>2-amino-8-naphthol-6-sulphonic acid<br>1:8-aminonaphthol-3:6-disulphonic acid<br>2-amino-8-naphthol-6-sulphonic acid<br>Do. | Beta-naphthol<br>Nitro-m-phenylenediamine<br>Beta-naphthol<br>Nitro-m-phenylenediamine<br>Salicylic acid<br>1:8-amino-naphthol-2:4-disulphonic acid<br>1-amino-8-naphthol-2:4-disulphonic acid<br>1-amino-8-naphthol-4-sulphonic acid<br>Beta-naphthol<br>Salicylic acid<br>2-amino-8-naphthol-6-sulphonic acid | Orange<br>Orange-red<br>Reddish-brown<br>Red<br>Bordeaux<br>Magenta<br>Blue-violet<br>Bronze-violet<br>Deep brown<br>Maroon<br>Prune 90 |
| 13        |                                                                                                                                                                                                                                                                                                              |                                                                                                                                                                                                                                                                                                                 | 85                                                                                                                                      |

Viscose as above unless otherwise



Invention is illustrated, without limiting the following examples in which the are by weight.

#### Example 1

dyebath is made up from 3000 parts of 20 parts of Glauber's salt, 3 parts of and 2 parts of the dyestuff obtained

Having now particularly described and ascertained the nature of my said invention and in what manner the same is to be performed, I declare that what I claim is:— 100

1. In the manufacture of dyed regenerated cellulose materials having an even level shade, the process which comprises applying to such regenerated cellulose materials a secondary disazo dyestuff having in the form of the free acid the probable formula: 105



wherein R<sub>1</sub> represents the coupled residue of a diazotized amine of the class consisting of chloraniline, amino-benzoic acid and anisidine, R<sub>2</sub> represents a naphthalene residue, and x is 1 or 2, thereby dyeing said regenerated cellulose materials in even level shades. 115

2. In the manufacture of dyed regenerated cellulose materials having an even level shade, the process which comprises applying to such regenerated cellulose materials a secondary disazo dyestuff having in the form of the free acid the probable formula: 120



wherein R<sub>3</sub> represents a coupled residue of an azo dye coupling component of the class 130

consisting of beta-naphthol, nitro-m-phenylene diamine, salicylic acid and amino-naphthol sulphonic acids,  $R_4$  represents Cl, an  $OCH_3$  or a  $COOH$  group and  $X$  represents hydrogen or a sulphonate group, thereby dyeing said regenerated cellulose materials in even level shades.

3. In the manufacture of dyed regenerated cellulose materials having an even level shade, the process which comprises applying to such regenerated cellulose materials a secondary disazo dyestuff having in the form of the free acid the probable formula:



20 wherein  $R_4$  represents a Cl, an  $OCH_3$  or a  $COOH$  group and  $x$  is 1 or 2, thereby dyeing said regenerated cellulose materials in even level shades.

25 4. As new products, regenerated cellulose materials dyed with disazo dyes having in the form of the free acid the probable formula:



wherein  $R_4$  represents a Cl, an  $OCH_3$  or a  $COOH$  group,  $R_2$  represents a naphthalene residue,  $R_3$  represents a coupled residue of an azo dye coupling component of the class consisting of beta-naphthol, nitro-m-phenylene diamine, salicylic acid and amino-naphthol sulphonic acids, and  $x$  is 1 or 2, the said dyed regenerated cellulose materials having even level shades.

35 5. As new products, regenerated cellulose materials dyed with disazo dyes having in the form of the free acid the probable formula:



40 wherein  $R_1$  represents a coupled residue of a diazotized amine of the class consisting of chlor-aniline, amino-benzoic acid and anisidine,  $R_2$  and  $R_3$  represent a naphthalene residue, and  $x$  is 1 or 2, the said dyed regenerated cellulose having even level shades.

45 6. As new products, regenerated cellulose materials dyed with disazo dyes having in the form of the free acid the probable formula:



wherein  $R_3$  represents a coupled residue of an azo dye coupling component of the class consisting of 2-amino-8-naphthol-6-sulphonic acid, nitro-phenylene-meta-diamine, beta-naphthol, and salicylic acid, and  $X$  represents hydrogen or a  $SO_3H$  group, the said dyed regenerated cellulose materials having even level shades.

70 7. As new products, regenerated cellulose materials dyed with disazo dyes having in the form of the free acid the probable formula:



80 wherein  $R_2$  represents a naphthalene residue,  $R_3$  represents a coupled residue of an azo dye coupling component of the class consisting of beta-naphthol, nitro-m-phenylene diamine, salicylic acid and amino-naphthol sulphonic acids and  $x$  is 1 or 2, the said dyed regenerated cellulose materials having even level shades.

85 8. As new products, regenerated cellulose materials dyed with disazo dyes having in the form of the free acid the probable formula:



95 wherein  $R_2$  represents a naphthalene residue,  $R_3$  represents a coupled residue of an azo dye coupling component of the class consisting of beta-naphthol, nitro-m-phenylene diamine, salicylic acid and amino-naphthol sulphonic acids and  $x$  is 1 or 2, the said dyed regenerated cellulose having even level shades.

100 9. As new products, regenerated cellulose materials dyed with disazo dyes having in the form of the free acid the probable formula:



110 wherein  $R_3$  represents a naphthalene residue, and  $x$  is 1 or 2, the said dyed regenerated cellulose having even level shades.

115 10. As new products, regenerated cellulose materials dyed with disazo dyes having in the form of the free acid the probable formula:



125 said dyed regenerated cellulose having even level shades.

11. As new products, regenerated cellulose materials dyed with disazo dyes having in the form of the free acid the probable formula:

the form of the free acid the probable formula:



15 the said dyed regenerated cellulose having even level shades.

12. As new products, regenerated cellulose materials dyed with disazo dyes having in the form of the free acid the probable formula:



30 wherein X represents H or a SO<sub>3</sub>H group, said dyed regenerated cellulose having even level shades.

13. As new products, regenerated cellulose materials dyed with disazo dyes having in the form of the free acid the probable formula:



wherein  $R_3$  represents a naphthalene residue,  $R_4$  represents chlorine or an alkoxy group, and  $x$  is 1 or 2, the said dyed regenerated cellulose having even level shades.

45 14. As new products, regenerated cellulose materials dyed with disazo dyes having in the form of the free acid the probable formula:



wherein R<sub>3</sub> represents a coupled residue of an azo dye coupling component of the class consisting of beta-naphthol, nitro-m-phenylene diamine, salicylic acid and amino-naphthol sulphonic acids, R<sub>4</sub> represents chlorine, a carboxylic or alkoxy group, and X represents H or SO<sub>3</sub>H group, the said dyed regenerated cellulose having even level shades.

35 15. As new products, regenerated cellulose materials dyed with disazo dyes having in



the said dyed regenerated cellulose having even level shades.

16. As new products, regenerated cellulose materials dyed with disazo dyes having in the form of the free acid the probable formula:



the said dyed regenerated cellulose having even level shades.

17. As new products, regenerated cellulose materials dyed with disazo dyes having the form of the free acid the probable formula:



wherein  $R_5$  represents chlorine or a  $OCH_3$  group, and  $R_6$  represents a coupled residue of an azo dye coupling component of the class consisting of beta-naphthol, nitro-m-phenylene diamine, salicyclic acid and amino-naphthol sulphonic acids, the said dyed regenerated cellulose having even level shades.

18. As new products, regenerated cellulose materials dyed with disazo dyes having in the form of the free acid the probable formula:



wherein  $R_4$  represents chlorine, or a  $\text{COOH}$  or  $\text{OCH}_3$  group, and  $R_8$  represents the coupled residue of an azo dye coupling component of the class consisting of beta-naphthol, nitro-phenylene-meta-diamine, salicylic acid, 2-amino-8-naphthol-6-sulphonic acid and 1:8 amino-naphthol-4-sulphonic acid, the said dyed regenerated cellulose having even level shades.

#### 19. As new products, regenerated cellulose 130

materials dyed with disazo dyes having in the in the form of the free acid the probable form of the free acid the probable formula: formula:



- 10 wherein  $R_6$  represents chlorine or a  $COOH$  group and  $X$  represents hydrogen or a  $SO_3H$  group, the said dyed regenerated cellulose having even level shades.

15 20. As new products, regenerated cellulose materials dyed with disazo dyes having in the form of the free acid the probable formula:



the said dyed regenerated cellulose having even level shades.

25. As new products, regenerated cellulose materials dyed with disazo dyes having in the form of the free acid the probable formula: 80



25 the said dyed regenerated cellulose having even level shades.

- even level shades.

21. As new products, regenerated cellulose materials dyed with disazo dyes having in the form of the free acid the probable formula:



wherein R<sub>6</sub> represents a OCH<sub>3</sub>, Cl or COOH group, and x is 1 or 2, the said dyed regenerated cellulose having even level shades.

26. As new products, regenerated cellulose materials dyed with disazo dyes having in the form of the free acid the probable formula:



85 wherein R<sub>6</sub> represents chlorine or a COOH group, the said dyed regenerated cellulose having even level shades.

- 10 having even lever shades.

22. As new products, regenerated cellulose materials dyed with disazo dyes having in the form of the free acid the probable formula:



wherein R<sub>5</sub> represents chlorine or a OCH<sub>3</sub> group, the said dyed regenerated cellulose having even level shades.

23. As new products, regenerated cellulose materials dyed with disazo dyes having in the form of the free acid the probable formula:



the said dyed regenerated cellulose having even level shades.

- 65 24. As new products, regenerated cellulose materials dyed with disazo dyes having

wherein  $R_3$  represents a naphthalene residue,  $R_4$  represents chlorine or an alkoxy group and  $\alpha$  is 1 or 2, the said dyed regenerated cellulose having even level shades.

27. In the manufacture of dyed regenerated cellulose materials having an even level shade the process which comprises applying to such regenerated cellulose material certain secondary disazo dyestuffs, said disazo dyestuffs having the probable formula:  $R_1 - N = N - R_2 - N = N - R_3$ , wherein  $R_1$  represents the alkaline-coupled residue of an amine of the benzene series of the class consisting of parachlor-aniline, meta-amino-benzoic acid and ortho-anisidine,  $R_2$  represents the alkaline-coupled residue of an amino-naphthol-sulphonic acid of the class consisting of 2-amino-5 naphthol-7-sulphonic acid, 2-amino-8 naphthol-6-sulphonic acid, 1-amino-5-naphthol-7-sulphonic acid, 1:8-amino-naphthol-3:6-disulphonic acid, the nitrogen of the amino group being one of the nitrogens forming part of the azo group between  $R_2$  and  $R_3$ , and  $R_3$  represents the coupled residue of an azo dye coupling component of the class consisting of beta-

naphthol, nitro-meta-phenylene-diamino, salicylic acid, 1:8-amino-naphthol-2:4-disulphonic acid, 1-amino-8-naphthol-4-sulphonic acid, and 2-amino-8-naphthol-6-sulphonic acid.

5 In testimony whereof I affix my signature.

RAINALD BRIGHTMAN.

**Certificate of Correction**

Patent No. 1,873,278.

August 23, 1932.

RAINALD BRIGHTMAN

It is hereby certified that error appears in the printed specification of the above-numbered patent requiring correction as follows: Page 1, lines 70 to 75, strike out the formula and insert instead:



and that the said Letters Patent should be read with this correction therein that the same may conform to the record of the case in the Patent Office.

Signed and sealed this 11th day of October, A. D. 1932.

[SEAL.]

**M. J. MOORE,**  
*Acting Commissioner of Patents.*

35

40

45

50

55

60

65

naphthol, nitro-meta-phenylene-diamino, salicylic acid, 1:8-amino-naphthol-2:4-disulphonic acid, 1-amino-8-naphthol-4-sulphonic acid, and 2-amino-8-naphthol-6-sulphonic acid.

5 In testimony whereof I affix my signature.

RAINALD BRIGHTMAN.

**Certificate of Correction**

Patent No. 1,873,278.

August 23, 1932.

RAINALD BRIGHTMAN

It is hereby certified that error appears in the printed specification of the above-numbered patent requiring correction as follows: Page 1, lines 70 to 75, strike out the formula and insert instead:



and that the said Letters Patent should be read with this correction therein that the same may conform to the record of the case in the Patent Office.

Signed and sealed this 11th day of October, A. D. 1932.

[SEAL.]

**M. J. MOORE,**  
*Acting Commissioner of Patents.*

35

40

45

50

55

60

65

**Certificate of Correction**

Patent No. 1,873,278.

August 23, 1932.

**RAINALD BRIGHTMAN**

It is hereby certified that error appears in the printed specification of the above-numbered patent requiring correction as follows: Page 1, lines 70 to 75; strike out the formula and insert instead:



and that the said Letters Patent should be read with this correction therein that the same may conform to the record of the case in the Patent Office.

Signed and sealed this 11th day of October, A. D. 1932.

[Signature.]

**M. J. MOORE,**  
Acting Commissioner of Patents.